

## 1

3,041,215

SOLUTIONS AND METHODS FOR FORMING  
PROTECTIVE COATINGS ON TITANIUM

Herbert Arthur Henry Jenkins and Dennis Brian Freedman, Brentford, England, assignors to Parker Rust Proof Company, Detroit, Mich., a corporation of Michigan

No Drawing. Filed Feb. 7, 1956. Ser. No. 563,865  
Claims priority, application Great Britain Feb. 7, 1955  
15 Claims. (Cl. 148—6.14)

This invention relates to the formation of adherent protective coatings on titanium and more particularly to chemically formed fluoride coatings on titanium and titanium base alloys.

It is an important object of the invention to provide improved solutions and methods for chemically forming strongly adherent coatings on surfaces of titanium and titanium base alloys.

Other important objects of the invention are to provide articles of titanium and of titanium alloys which have formed thereon characteristic corrosion resistant coatings and to provide said articles in such coated form whereby they may be deformed and cold worked without injury to the substrate.

The above and other objects of the invention will become apparent during the course of the following description.

In accordance with the invention, titanium and titanium base alloys can be provided with a uniform, adherent fluoride coating which facilitates drawing and cold working of the metal and which imparts thereto superior corrosion resistance. Formation of the coating occurs from contacting a surface of the metal with an aqueous acidic solution containing the fluoride ion and ions of one or more of the alkali metals. For purposes of the present invention, ammonium is included in the term alkali metals. It is essential that a pH between about 2 and 6 be maintained for the solution and preferably the pH is maintained between about 2.5 and 5.

It has now been found that a certain group of compounds have in common the unusual effect of reacting with titanium and titanium base alloys in the presence of the fluoride ion and the ions of the alkali metals to form an exceptionally superior and, from what appears, a type of complex fluoride coating. The precise chemical nature of the coating remains unknown, but it is known from its properties and effects to be exceptionally adherent and protective and to be characteristic of solutions having the mentioned ingredients and one of the compounds of this certain group. The distinct advantages of the invention are realized only under the conditions that the predominant part and preferably all of the acidity of the solution is derived from one of this certain group of compounds.

Also according to the invention, this certain group of compounds are all acids and all exhibit to a marked degree the described beneficial property when used in the type solutions mentioned as the principal source of acidity. The group of acids so found to exhibit this property comprises for one, hydrofluoric acid which has its own distinct advantages as will appear, and also hydrochloric acid, nitric acid, and sulphuric acid which exhibit like effects and similarly their use has separate advantages. Discovered to be substantially equivalent of the foregoing inorganic acids in their effect on coating but also having separate advantages are organic acids which have a primary dissociation constant less than  $3 \times 10^{-2}$  but greater than  $1 \times 10^{-6}$ . By primary dissociation constant is meant the dissociation constant measured at approximately room temperature for the first hydrogen atom when there are more than one dissociable hydrogen atoms. Of the latter acids, i.e., the organic acids, which are useful for forming

## 2

coatings of the present invention, the following are preferred: succinic acid; maleic acid; salicylic acid; tartaric acid; phthalic acid; acetic acid; benzoic acid; and citric acid.

According to a feature of the invention, advantages are realized when solid materials are used as the source of one or more of the above group of acids and/or the other ingredients of the solutions. The solid compositions are much less corrosive than the solutions so that packaging and handling are facilitated, and economies in storage and transportation are effected.

The coatings of the invention are formed by contacting the surface of titanium and the like with an aqueous solution containing one or more of the acids of the above

15 group, viz., hydrofluoric acid, and hydrochloric acid, nitric acid or sulphuric acid and an organic acid having a primary dissociation constant less than  $3 \times 10^{-2}$  but greater than  $1 \times 10^{-6}$  at a pH between 2 and 6; the solution also containing at least 0.5% fluoride ions and at least 0.5%  
20 sodium or potassium ions or both. Preferably the concentration of the above group of acids is maintained so that the pH of the solution is within the optimum range of 2.5 to 5. The anion radical of these acids which dissociates from the hydrogen radical appears to be the most  
25 important factor accounting for the similarity in effect on coating of these acids when present in the solution, and consequently while impurities including other acids may be present in minor amounts, it is imperative that the greater part, and preferably all of the acidity of the solution  
30 is derived from one or more of the acids of the above group.

It has been found that the coatings obtained with solutions containing sodium are formed more rapidly than those obtained with solutions containing potassium. If  
35 ammonium or lithium ions or both are used in place of sodium or potassium, their concentration must be substantially increased, and, in the case of ammonium, the concentration of the ammonium ion should be at least 2%. In the case of lithium, it is preferable to use at least 2%  
40 but it is possible to use less. Unless otherwise indicated, percentages as given throughout the specification are by weight percent. Mixtures of the above alkali metals may be used and in this case the minimum concentration will lie somewhere between the minimum concentrations given  
45 above for the ions separately depending on the relative proportions of each in the mixture. Excellent coatings have been formed from concentrations of 8% alkali metal ion.

The solution preferably should be substantially free from calcium and other ions known to form fluorides that  
50 are insoluble in aqueous solutions as otherwise waste of the fluoride ion occurs by allowing them to be precipitated as simple insoluble fluorides. However, such ions can be tolerated in the amounts usually found in tap water, and consequently this water may be used for preparing the solutions. Using the solutions with the above group of acids present in the strengths mentioned, the concentration of the fluoride ion must be at least 0.9% and can be used in quantities below and above saturation which is approximately of the order of 10% fluoride ion.  
60 The preferred range of concentration of the fluoride ion has been found to be between about 0.9% to 8%.

Articles may be treated either by spraying or by immersion and in handling of the solutions rubber or polythene-lined containers are recommended as the solutions are corrosive.

Entirely satisfactory coatings can be formed without any activation or chemical pretreatment of the titanium surfaces. However, it is oftentimes advantageous first to pickle the surface with a solution containing hydrofluoric and nitric acids. A 5% hydrofluoric acid solution has been found to be a useful pickle. In some cases the

nature of the pickle solution may be a factor in obtaining the most successful coating and in such cases its nature must be determined by the particular titanium alloy to be processed. Any grease that may be present on the surface as received for coating will generally be removed by this pickling, but if necessary, a preliminary degreasing treatment may also be applied. If the titanium has been annealed it may carry a heavy scale, and this, of course, should be removed also.

From the evidence that is available, the coating action of these solutions appears to be the result of the formation of a thin layer of solution saturated with titanium at the surface thereof under treatment. Accordingly, when a fresh solution is brought into contact with the metal surface there is a time lag before coating starts while the titanium metal is being dissolved from the surface. It is therefore preferred to add titanium to the solution. It has been found that this can be accomplished conveniently by adding to the solution just prior to immersion of the metal enough fluotitanate compound to saturate the solution and simple tests under operating conditions can be made to determine the amount required in a particular operation. A fluotitanate compound such as an alkali fluotitanate, as for example, potassium fluotitanate can also be included in the coating solution initially and it can be mixed with the solid compositions previously mentioned for making up the solutions.

The solutions can be prepared by dissolving three ingredients in water, viz., one of the above group of acids, a fluoride and an alkali metal compound and in the case of hydrofluoric acid, two ingredients, viz., the acid and an alkali metal compound. Alternatively, in the case of the other acids, two ingredients can also be used, viz., the acid and an alkali metal fluoride.

With respect to the above group of acids, while they are substantially equivalent in their effect on the type of coating formed, each or certain of the acids of the group have specific advantages when used in the solution alone and this property of certain of the acids makes natural subgroupings from the above group of acids. The use of hydrofluoric acid without the others of the group in the solution as the predominant or sole source of the acidity thereof has the additional advantage that the complex fluoride coating formed does not contain any other acid or salt thereof entrained or otherwise carried over from the solution. The main advantage (in addition, of course, to those described for the group as a whole) in using alone the other mineral acids, namely, hydrochloric, nitric and sulphuric acid, is that they are cheap and readily available. The advantage of the use of the organic acids having a dissociation constant as set forth above without the others as the sole source of the acidity of the solution is that the control required to maintain the pH within the required range is simpler.

Hereinafter, the invention will be described with respect to each of the above subgroups of the acids of the general group. In the case of hydrofluoric acid, the solution can be prepared by dissolving in water the acid and an alkali metal compound. Alternatively, a solution of an alkali metal bifluoride can be used to provide the essential constituents of this solution. In accordance with the feature of the invention wherein solid materials are employed to facilitate storage and transportation, a solid composition can be made by mixing a solid bifluoride and a solid compound of an alkali metal which when dissolved in water, or in an aqueous solution, will provide a working solution. If the cation of the solid bifluoride is an alkali metal, a single solid compound can be used for this solution which makes the process extremely simple and convenient. For example, a 15% solution made from solid potassium bifluoride and a 12% solution made from solid sodium bifluoride each produced a strongly adherent brown-gray coating on titanium.

In the case of the other mineral acids, hydrochloric,

nitric and sulphuric acid, the solution can be prepared from three ingredients, viz., one of these acids, a fluoride and an alkali metal. Alternatively, one of these acids and an alkali metal fluoride only need be used to supply the solution. Advantageously, a solid composition can be used as the source of these acids and this feature will be illustrated with respect to sulphuric acid. In the case of sulphuric acid, a bisulphate or sulphamic acid can be used as the source of sulphuric acid in the solution. As these are solids, their use has advantages and an example of such a composition comprises a solid mixture of a solid bisulphate or sulphamic acid, a solid fluoride and a solid alkali metal compound. This will provide a working solution when dissolved in water or an aqueous solution. An even simpler solid mixture comprises two compounds, e.g., a bisulphate and an alkali metal fluoride. Good results were obtained from a solution prepared from a mixture which comprises 5 parts by weight of solid sodium bisulphate and 4 parts by weight of solid sodium fluoride which is dissolved in water in the quantity of 9 parts by weight of the mixture to make 100 parts by weight of solution.

In the case of the organic acids which have a dissociation constant between  $1 \times 10^{-6}$  and  $3 \times 10^{-2}$ , the solutions to be brought into contact with the metal surface can be prepared by dissolving in water three ingredients, namely, the organic acid, a compound yielding fluoride ions and an alkali metal compound. If desired, two ingredients can be used, namely, the acid and an alkali metal fluoride. Either a solution ready for use or a concentrate which is diluted just prior to use can be prepared. As some of the organic acids, e.g., citric and tartaric acids, are solids their use in such form provides the advantages previously set forth for the solid materials. A solid composition according to this feature of the invention comprises a mixture of a solid organic acid having a primary dissociation constant between  $1 \times 10^{-6}$  and  $3 \times 10^{-2}$  with a solid of one or more of the compounds providing the fluoride ion and the alkali metal ion when dissolved. Even greater simplification of the process arises from the use of a solid mixture which consists of only two compounds, as for example, citric acid and sodium or potassium fluoride.

The following examples illustrate the improved acid fluoride coating solutions of the present invention and method of applying these solutions to surfaces of titanium, and are given with respect to each of the above subgroups of acids, namely, hydrofluoric acid, and the mineral acids, hydrochloric, nitric and sulphuric acid, and the organic acids.

#### Example 1

Coatings were produced on titanium by the various hydrofluoric acid or hydrofluoric acid-producing solutions set forth below by pickling titanium panels for 30 seconds in a solution of nitric acid and hydrofluoric acid, rinsing them and then immersing them in the various solutions at room temperature until gassing stopped. The solutions and the coating weights obtained were:

|    | Solution                                                             | Time to cessation of gassing, Minutes | Coating Weight, mg./sq. ft. |
|----|----------------------------------------------------------------------|---------------------------------------|-----------------------------|
| 65 | 15.6% $\text{KHF}_2$                                                 | 2                                     | 1,220                       |
|    | 7.8% $\text{KHF}_2 + 0.1\% \text{K}_3\text{TiF}_6$                   | 15                                    | 2,750                       |
|    | 11.6% $\text{KF} + 0.1\% \text{HF}$                                  | 20                                    | 895                         |
|    | 5.8% $\text{KF} + 0.04\% \text{HF}$                                  | 25                                    | 286                         |
| 70 | 4% $\text{KHF}_2 + 1\% \text{NaHF}_2 + 0.1\% \text{K}_3\text{TiF}_6$ | 3                                     | 627                         |
|    | 12% $\text{NaHF}_2$                                                  | 2                                     | 900                         |

The following examples are of coating solutions containing the mineral acids subgroup; sulphuric acid being chosen as representative thereof.

## Example 2

The solution consisted of:

|                     | Percent |
|---------------------|---------|
| $H_2SO_4$           | 1.5     |
| KF                  | 5       |
| $NaNO_3$            | 0.25    |
| $K_2TiF_6$          | 0.1     |
| Water to make 100%. |         |

A coating having good adhesion and dark gray in appearance was produced in 2½ minutes at 20° C.

## Example 3

The solution consisted of:

|                     | Percent |
|---------------------|---------|
| $KHSO_4$            | 7       |
| KF                  | 5       |
| $NaNO_3$            | 0.25    |
| $K_2TiF_6$          | 0.1     |
| Water to make 100%. |         |

The same product was used as in the above example and the same results were obtained.

## Example 4

The solution consisted of:

|                     | Percent |
|---------------------|---------|
| $NaHSO_4$           | 5       |
| KF                  | 5       |
| $NaNO_3$            | 0.25    |
| $K_2TiF_6$          | 0.1     |
| Water to make 100%. |         |

A coating having good adhesion and of medium gray appearance was produced in 2 minutes at 20° C.

## Example 5

The solution consisted of:

|                     | Percent |
|---------------------|---------|
| $NaHSO_4$           | 5       |
| NaF                 | 4       |
| Water to make 100%. |         |

A coating having very good adhesion and of medium gray appearance was produced in 4 minutes at 20° C., in 1 minute at 38° C., in 20 seconds at 72° C., and in 7 seconds at 95° C.

In each of the examples from 2-5, commercially pure titanium wire was successfully drawn from a diameter of 0.160 inch to 0.0124 inch through a sequence of dies. The surface of the wire remained in good condition during the drawing operation.

The following examples are of coating solutions containing organic acids having a dissociation constant within the limits set forth above.

## Example 6

The solution consisted of:

|                     | Percent |
|---------------------|---------|
| Citric acid         | 7       |
| Potassium fluoride  | 10      |
| Water to make 100%. |         |

Dark adherent coatings were formed on titanium in 5 minutes at 20° C.

## Example 7

The solution consisted of:

|                     | Percent |
|---------------------|---------|
| Phthalic acid       | 5       |
| Potassium fluoride  | 10      |
| Water to make 100%. |         |

Dark adherent coatings were formed on titanium in 5 minutes at 20° C.

## Example 8

The solution consisted of:

|                     | Percent |
|---------------------|---------|
| Acetic acid         | 48      |
| Potassium fluoride  | 6       |
| Water to make 100%. |         |

Dark gray coatings of good adhesion were formed on titanium in 5 minutes at 20° C.

It will thus be seen that there has been provided by this invention, an article, a composition and a method in which the various objects hereinabove set forth, together with many thoroughly practical advantages are successfully achieved.

Since certain changes may be made in the above invention and different embodiments of the invention may be made without departing from the scope thereof, it is intended that all matter contained in the above-described disclosure shall be interpreted as illustrative and not in a limiting sense.

What is claimed is:

1. An aqueous acidic solution for producing a coating on surfaces of titanium and titanium base alloys having a pH between 2 and 6 and consisting of at least about 0.5% of the fluoride ion, at least about 0.5% of the ions of at least one of the alkali metals, and an acid selected from the group consisting of hydrofluoric acid, hydrochloric acid, nitric acid, and sulphuric acid, the concentration of said acid in the solution being such that the predominant part of the acidity of the solution is derived from said acid.

2. An aqueous acidic solution for producing a coating on surfaces of titanium and titanium base alloys having a pH between 2 and 6 and consisting of at least about 0.5% of the fluoride ion, at least about 0.5% of the ions of at least one of the alkali metals, and an acid selected from the group consisting of hydrofluoric acid, hydrochloric acid, nitric acid, and sulphuric acid, the concentration of said acid in the solution being such that the predominant part of the acidity of the solution is derived from said acid.

3. An aqueous acidic solution for producing a coating on surfaces of titanium and titanium base alloys having a pH between 2 and 6 and consisting of about 0.9% to 8% fluoride ion, at least about 0.5% ions of at least one of the alkali metals, and hydrofluoric acid, the concentration of said acid in the solution being such that the predominant part of the acidity of the solution is derived from said acid.

4. An aqueous acidic solution for producing a coating on surfaces of titanium and titanium base alloys having a pH between 2 and 6 and consisting of about 0.9% to 8% fluoride ion, at least about 0.5% ions of at least one of the alkali metals, and hydrochloric acid, the concentration of said acid in the solution being such that the predominant part of the acidity of the solution is derived from said acid.

5. An aqueous acidic solution for producing a coating on surfaces of titanium and titanium base alloys having a pH between 2 and 6 and consisting of about 0.9% to 8% fluoride ion, at least about 0.5% ions of at least one of the alkali metals, and nitric acid, the concentration of said acid in the solution being such that the predominant part of the acidity of the solution is derived from said acid.

6. An aqueous acidic solution for producing a coating on surfaces of titanium and titanium base alloys having a pH between 2 and 6 and consisting of about 0.9% to 8% fluoride ion, at least about 0.5% ions of at least one of the alkali metals, and sulphuric acid, the concentration of said acid in the solution being such that the predominant part of the acidity of the solution is derived from said acid.

7. A solid composition soluble in water so as to form a solution capable of producing an adherent coating on surfaces of titanium and titanium base alloys consisting essentially of a mixture of a bifluoride, an alkali metal compound, and a fluoritanate in an amount sufficient to

saturate said solution, the proportions of said bifluoride, alkali metal compound and fluotitanate being such as to produce an aqueous acidic solution having a pH between 2 and 6 and containing at least 0.5% of the fluoride ion and at least 0.5% of the alkali metal ion.

8. A solid composition soluble in water so as to form a solution capable of producing an adherent coating on surfaces of titanium and titanium base alloys consisting of a mixture of at least one compound of the group sulphamic acid and a bisulphate, a fluoride, and an alkali metal compound, the proportions of said acid, fluoride, and alkali metal compound being such as to produce an aqueous acidic solution having a pH between 2 and 6 and containing at least 0.5% of the fluoride ion and at least 0.5% of the alkali metal ion.

9. A solid composition soluble in water so as to form a solution capable of producing an adherent coating on surfaces of titanium and titanium base alloys consisting essentially of a mixture of at least one compound of the group sulphamic acid and a bisulphate, a fluoride, an alkali metal compound, and a fluotitanate in an amount sufficient to saturate said solution, the proportions of said acid, fluoride, and alkali metal compound being such as to produce an aqueous acidic solution having a pH between 2 and 6 and containing at least 0.5% of the fluoride ion and at least 0.5% of the alkali metal ion.

10. A method for producing an adherent coating on the surfaces of titanium and titanium base alloys comprising subjecting said surfaces to the action of an aqueous acidic solution having a pH between 2 and 6 and consisting of at least about 0.5% of the fluoride ion, at least about 0.5% of the ions of at least one of the alkali metals, and an acid selected from the group consisting of hydrofluoric acid, hydrochloric acid, nitric acid, and sulphuric acid, the concentration of said acid in the solution being such that the predominant part of the acidity of the solution is derived from said acid.

11. A method for producing an adherent coating on the surfaces of titanium and titanium base alloys comprising subjecting said surfaces to the action of an aqueous acidic solution having a pH between 2 and 6 and consisting of about 0.9% to 8% of the fluoride ion, at least about 0.5% of the ions of at least one of the alkali metals, and hydrofluoric acid, the concentration of said acid in the solution being such that the predominant part of the acidity of the solution is derived from said acid.

12. A method for producing an adherent coating on the surfaces of titanium and titanium base alloys comprising subjecting said surfaces to the action of an aqueous acidic solution having a pH between 2 and 6 and

consisting of about 0.9% to 8% of the fluoride ion, at least about 0.5% of the ions of at least one of the alkali metals, and hydrochloric acid, the concentration of said acid in the solution being such that the predominant part of the acidity of the solution is derived from said acid.

13. A method for producing an adherent coating on the surfaces of titanium and titanium base alloys comprising subjecting said surfaces to the action of an aqueous acidic solution having a pH between 2 and 6 and consisting of about 0.9% to 8% of the fluoride ion, at least about 0.5% of the ions of at least one of the alkali metals, and nitric acid, the concentration of said acid in the solution being such that the predominant part of the acidity of the solution is derived from said acid.

15. A method for producing an adherent coating on the surfaces of titanium and titanium base alloys comprising subjecting said surfaces to the action of an aqueous acidic solution having a pH between 2 and 6 and consisting of about 0.9% to 8% of the fluoride ion, at least about 0.5% of the ions of at least one of the alkali metals, and sulphuric acid, the concentration of said acid in the solution being such that the predominant part of the acidity of the solution is derived from said acid.

15. An article of manufacture having a substrate consisting of a metal of the group titanium and titanium base alloys, a complex fluoride coating uniformly distributed over and strongly adhering to said substrate, said fluoride coating being the reaction product between said metal and a solution having a pH between 2 and 6 and consisting of at least about 0.5% of the fluoride ion, at least about 0.5% of the ions of at least one of the alkali metals, and an acid selected from the group consisting of hydrofluoric acid, hydrochloric acid, nitric acid, and sulphuric acid, the concentration of said acid in the solution being such that the predominant part of the acidity of the solution is derived from said acid.

#### References Cited in the file of this patent

#### UNITED STATES PATENTS

|    |           |               |       |               |
|----|-----------|---------------|-------|---------------|
| 40 | 2,489,152 | Panepinto     | ----- | Nov. 22, 1949 |
|    | 2,550,660 | Amundsen      | ----- | May 1, 1951   |
|    | 2,711,364 | Beach         | ----- | June 21, 1955 |
|    | 2,864,732 | Miller et al. | ----- | Dec. 16, 1958 |

#### OTHER REFERENCES

- "Final Report on Chem. Surface Treatment of Titanium in Watertown Arsenal" by Battelle Memorial Institute, October 30, 1953, 30 pages.
- Am. Machinist, June 11, 1951, p. 152.